

## UNITED STATES PATENT OFFICE.

GIOVANNI TAGLIANI, OF BASEL, SWITZERLAND, ASSIGNOR, BY MESME ASSIGNMENTS, TO CHEMICAL WORKS, FORMERLY SANDGZ, OF BASEL, SWITZERLAND, A JOINT-STOCK COMPANY.

## PROCESS FOR TREATING COTTON OR OTHER THREADS CONTAINING CELLULOSE.

No Drawing. Application filed June 29, 1925, Serial No. 40,452, and in Germany July 3, 1924.

The present invention relates to improvements in a process of treating cotton or other cellulose fibers in order to render them indifferent to substantive dyestuffs.

It is known that vegetable fibers can be rendered indifferent to substantive dyestuffs by treating them after an alkalization with carbon acid chlorides, preferably in the presence of indifferent organic solvents. This process has, however, the disadvantage of being relatively expensive owing to the acid chlorides which have to be used, and, moreover, the cellulose compound thus obtained is not resistant to various agents used in the treatment of textile fibers, especially to alkalies and to high temperatures.

Further, a process has been described for rendering uncolored cellulose fibers, or such which have been dyed in the vat, indifferent to substantive dyestuffs, by alkalizing them and treating them afterwards with sulphonate chlorides of the aromatic series, whereby these aromatic sulphonate chlorides are preferably used in the presence of indifferent organic solvents. This process has essential advantages compared with the above-mentioned process, which consists in that cheap esterifying agents can be employed, and that the cellulose compounds obtained by means of the aromatic sulphonate chlorides are more stable against alkalies and other agents and against high temperatures than those obtained by means of aromatic carbonic chlorides.

In further improvement of this last mentioned process I have found that cellulose fibers, loose or in the shape of threads, or as woven fabric, preliminarily dyed with substantive dyestuffs, can be rendered indifferent against other substantive dyestuffs.

## Example.

Cotton yarn, dyed with a substantive dyestuff is alkalized by treating it for a certain time in a 14% alcoholic solution of caustic soda. The thus treated yarn is then withdrawn and hydroextracted to remove an excess of lye.

1 kg. of the alkalized yarn is then immersed in a resistant vessel, containing 15

litres of a 20% solution of paratoluene sulphonate chloride in tetrachloride of carbon. After a short time the reaction takes place and the temperature rises, without the boiling point of the liquid being reached. It is important that the yarn is always wholly immersed. Thereupon the whole is allowed to cool down for several hours, and is then heated again until the boiling point of the liquid is nearly reached. The yarn is then removed, hydroextracted and afterwards soaped several times in a bath at about 60° C. until the smell of carbon tetrachloride and paratoluene sulphonate chloride has almost completely disappeared. The fibres are then hydroextracted and dried. The thus obtained fibres resist all the usual agents of the textile industry, such as acids, alkalies and reducing agents.

To alkalize the dyed vegetable fibres, caustic potash may be used instead of caustic soda. Tetrachloride of carbon may be replaced by any other indifferent organic solvent, such as the halogenized hydrocarbons of the aliphatic series, further hydrocarbons of the petroleum series and particularly benzol and its homologues. Paratoluene sulphonate chloride may be replaced as esterifying agent by another aromatic sulphonate chloride, for instance benzene sulphonate chloride, ortho toluene sulphonate chloride, xylene sulphonate chloride and naphthalene sulphonate chlorides, as well as their halogen derivatives.

## I claim—

1. A process of rendering cellulose fibres, preliminarily dyed with substantive dyestuffs, indifferent to substantive dyestuffs, which comprises alkalizing the dyed fibres and treating them with aromatic sulphonate chlorides.

2. A process of rendering cellulose fibres, preliminarily dyed with substantive dyestuffs, indifferent to substantive dyestuffs, which comprises alkalizing the dyed fibres and treating them with para toluene sulphonate chloride.

In testimony whereof, I have signed my name to this specification.

GIOVANNI TAGLIANI.